

E. M. CHADBOURNE.  
OILED CONCRETE ROADWAY.  
APPLICATION FILED AUG. 4, 1909.

956,940.

Patented May 3, 1910.



Witnesses.

*O. H. Young*  
*W. H. Pinfield*

Inventor:

Edward M. Chadbourne  
By *Gen. H. Young*  
*His Attorney*

# UNITED STATES PATENT OFFICE.

EDWARD M. CHADBOURNE, OF SAN FRANCISCO, CALIFORNIA.

## OILED CONCRETE ROADWAY.

956,940.

Specification of Letters Patent.

Patented May 3, 1910.

Application filed August 4, 1909. Serial No. 511,169.

*To all whom it may concern:*

Be it known that I, EDWARD M. CHADBOURNE, citizen of the United States, residing in the city and county of San Francisco 5 and State of California, have invented new and useful Improvements in Oiled Concrete Roadways, of which the following is a specification.

This invention relates to highway construction, and pertains especially to an oiled reinforced cement macadam road.

The object of the invention is to provide a road, street or way which is strong structurally, monolithic in character, and with a 15 wearing cushion on the surface which is dustless, permanent, and requiring little or no expense for maintenance or repair.

The special object of the present invention is to so construct this roadway that this 20 surface cushion, which is made up of a mixture of oil and screenings, is firmly anchored to its underneath foundations; and in the construction of this roadway provision is made to prevent the downward percolation 25 of the oil, so that in the end a true asphaltic surface for the roadway is produced.

The invention consists of the parts and the construction and combination of parts as hereinafter more fully described and claimed, 30 having reference to the accompanying drawings, in which—The figure is a sectional view in perspective, showing the method of constructing a roadway according to the invention.

In the practice of the invention, the road is graded, crowned and laid out, according to surveyed lines, and suitably prepared until it is compacted to a smooth hard surface. This preparation usually comprises the harrowing 35 of the road until about two inches of the surface is loose. It is then watered to a point of saturation and allowed to dry until it is no longer sticky or plastic, whereupon it is rolled or tamped until the surface is smooth and hard. Next the reinforcing fabric 40 is laid on the prepared sub-grade A. This reinforcing fabric consists preferably of a square mesh, with redrawn steel wires running longitudinally and laterally and 45 suitably connected by clips or locks 3. This fabric preferably has a 6x6 mesh, and is suitably supported on the sub-grade A so that it will lie about one inch above the sub-grade. This support for the reinforcing 50 fabric 2 is here shown as comprising a series of metal strips 4 punched out to form open-

ings 5, and having base flanges 6 bent in opposite directions, so that it will stand up edgewise on the sub-grade and in appearance be like an inverted T. These strips extend 60 at suitable intervals across the roadway, and also act as a reinforcement, since the openings 5 permit of a perfect bond of the concrete 7 on all sides of the reinforce and metal support. 65

After the reinforcing fabric is laid, the cement macadam 7 is placed as ordinary concrete, usually about four inches in thickness, and comprises proper mixtures of cement, sand, and crushed rock or gravel. The 70 crushed rock or gravel should be clean, and of such sizes as will pass through a two inch ring. This cement macadam is thoroughly mixed by a rotary concrete mixer, and sufficient water is added to produce a plastic 75 mixture, in which condition it is deposited on the prepared sub-grade and spread evenly thereover.

Before the cement macadam concrete layer 7 has set, and while it is still in a plastic 80 condition, it is covered with a course of clean hard rock of about egg size, as represented at 8. This course of heavy rock is spread evenly over the surface of the concrete and will become partially embedded in the same; 85 and when the concrete is set, this course of rock 8 will form an integral part of the concrete foundation, with the points projecting about an inch above the surface of the underneath concrete body in which the rock 90 is embedded. This roughened dressing 8 is one of the important features of this invention, because the interstices which are formed between the projecting pinnacles constitute little reservoirs of an inch or so 95 in depth in which the heavy asphaltic oil which is later applied will collect.

When the cement macadam and its rough surfacing 8 are thoroughly set and dried out, so that the course of heavy rock 8 is 100 integrally bonded with the underneath foundation, I apply a heavy asphaltic road oil, or heavy crude oil of asphaltic base. This oil is first heated to a temperature of about 200° Fahrenheit, so as to render it 105 limpid, and while at this temperature it is spread and brushed over the surface of the cement macadam, care being taken that all the interstices in the surface are thoroughly filled. If it were not for the pockets or 110 reservoirs formed by the protruding points 8 the oil would run off of the foundations,

and thus defeat one essential feature of the invention. Immediately after the oil has been applied, a layer of fine screenings is spread over the surface to a depth of about one inch. This layer of screenings sinks down into the oil pockets and absorbs the oil. This layer of oil-saturated screenings, represented at 10, is then rolled with a six ton, or heavier roller until it is compacted into what is, in actual effect, an asphaltic surface similar to the standard asphaltic pavements of to-day.

On account of the impervious character of the concrete, the oil in the small reservoirs or openings formed between the rocks of the layer 8 is within less than two inches of the surface, so that the oil deposited in these pockets has a chance to become thickened by evaporation or oxygenation, and the absorption of the heavy asphaltic residuum by the fine screenings gives durability and hardness to the surface. This desired change in the oil would not take place if the underneath foundation were porous so that the oil could sink through to three or six inches in depth.

In my construction the oil is kept and maintained near the surface, so that its whole bonding and elastic value is preserved and utilized.

30 The course of egg-sized rock 8 which is embedded in the top of the concrete is also in some cases part of the wearing surface, projecting up through the final asphaltic top dressing 10, and preventing slipping of 35 horses' feet on the asphaltic surface.

It is readily seen that the top layer of the asphaltic oil and screenings 10 is held very rigidly to the top of the concrete foundation, both by the adhesion of the oil to the 40 concrete and the top course 8, and the lock or bond formed by the pockets between the rocks of the course 8.

A roadway of this character has all the desired requisites of permanency provided 45 by the reinforced cement macadam foundation. It has all the elastic qualities of, and much greater durability than, the ordinary bituminized or asphalt street or roadway. And furthermore, it can be laid down for 50 from 25% to 50% cheaper, as practice has shown, than the ordinary asphalt or bituminized road.

Having thus described my invention, what I claim and desire to secure by Letters 55 Patent is—

1. The method of roadway construction which consists in preparing a suitable sub-

grade and spreading a suitable layer of concrete thereover, and while this concrete is still in a plastic condition covering it with 60 coarse rock thereby forming pockets in the top surface thereof, allowing the concrete with its rock coating to set into a solid structure, oiling the surface of the foundation so formed, so as to fill the pockets with 65 oil of asphaltic base, then applying a layer of screenings to the oil sufficient to take up the oil, and then subjecting the oiled surface to pressure.

2. The method of roadway construction 70 which comprehends preparing a suitable concrete foundation for the roadway, which foundation comprises a concrete slab extending over the roadway, and while this concrete is still in a plastic condition, forming pockets, of approximately an inch or more in depth on its surface, filling these pockets with a heavy asphaltic oil and then applying fine screenings to absorb the oil in the pockets, and rolling the plastic mixture so formed to compact the same in the pockets.

3. The method of constructing a cement macadam roadway consisting of placing a 85 layer of reinforced concrete on the sub-grade and while in a plastic condition providing its surface with oil retaining pockets, pouring a coating of heavy asphaltic oil over the 90 surface to fill the pockets, and spreading a layer of fine screenings over the oil to absorb the oil.

4. The method of roadway construction which comprises the following steps in substantially the following order, to-wit: first, the preparation of a suitable sub-grade; 95 second, the laying of a suitable concrete slab over this sub-grade and forming in the top of this slab pockets of approximately an inch or more in depth; third, filling these pockets with a heavy oil, which oil is normally in condition to be absorbed at ordinary temperatures; and fourth, spreading a 100 layer of screenings over the oiled surface of the road-bed, said layer of screenings being approximately an inch in thickness, and causing the screenings to sink into the oil in the pockets and fill the pockets.

In testimony whereof I have hereunto set my hand in the presence of two subscribing witnesses.

EDWARD M. CHADBOURNE.

Witnesses:

CHARLES EDELMAN,  
C. C. COOK.